# EUROPEAN PATENT APPLICATION

(11) **EP 4 786 632 A1**
(43) Date of publication of application: **05.08.2026**
(21) Application number: 24870971.9
(22) Date of filing: 27.09.2024
(51) Int. Cl.: C22C 38/44, C22C 38/40, C22C 38/18

(54) **HIGH-STRENGTH CHAIN STEEL, HIGH-CORROSION-RESISTANCE ORE CHAIN AND MANUFACTURING METHOD THEREFOR**

(30) Priority: 28.09.2023 CN 202311283446
(71) Applicant: BAOSHAN IRON & STEEL CO., LTD., Shanghai 201900 (CN)
(72) Inventor: ZHAO, Sixin, Shanghai 201900 (CN); WANG, Chengquan, Shanghai 201900 (CN)
(74) Representative: Tergau & Walkenhorst Intellectual Property GmbH
(86) International application number: PCT/CN2024/121788
(87) International publication number: WO 2025/067434

(57) **Abstract**

The present disclosure provides a high-strength chain steel, a high-corrosion-resistance mining chain, and a manufacturing method therefor. The chain steel comprises the following chemical elements in mass percentage: C: 0.20-0.30%, Si: 0.05-0.6%, Mn: 1.0-1.8%, Cr: 0.4-0.8%, Ni: 0.6-1.2%, Mo: 0.5-0.9%, Ti: 0.01-0.03%, Al: 0.02-0.05%, B: 0.001-0.005%, N: 0.002-0.006%, and the balance being Fe and inevitable impurities. The high-corrosion-resistance mining chain of present disclosure has both high strength and good corrosion resistance, and can be widely used in environments with a large amount of corrosive medium, such as engineering machinery, mines, ships, and marine engineering.

## Description

### TECHNICAL FIELD

The present disclosure relates to the technical field of high-strength chain steel and chain, in particular to a high-strength chain steel, a high-corrosion-resistance mining chain and a manufacturing method therefor.

### BACKGROUND

Approximately 1/6 of the global annual steel output is lost due to corrosion. In China, the direct economic losses caused by steel corrosion exceed 10 billion CNY annually. Furthermore, steel corrosion reduces the service life of steel structures, causes casualties and economic losses, and contributes to environmental pollution through emissions. Mining round link chains are crucial components for mechanized coal mining underground in coal mines, primarily serving as transmission chains on scraper conveyors, stage loaders, shearers and coal ploughs. They are required to have high strength and toughness, fatigue resistance, wear resistance and other properties during service. At present, the mining round link chain steels commonly adopted in the coal mining industry are generally the grades of mining chain steels specified in GB/T 10560-2017 "Steels for welded round link chains for mines", among which the high-strength mining round link chain steels most widely applied are mainly grades such as 23MnNiMoCr54 steel (abbreviated as 54 steel). Moreover, in response to the needs in practical applications, major steel mills in China have also developed a series of high-strength mining chain steels according to the different requirements of downstream users.

CN Patent Literature CN110714164A (published on January 21, 2020, entitled "High-Quality Cr54 Steel for Coal Mine Chain Links and Manufacturing Method therefor") discloses a high-quality 54 steel for coal mine chain links. By introducing the carbon equivalent, cold crack sensitivity coefficient and hot crack sensitivity coefficient, it ensures the weldability of the chain steel and improves the cold/hot brittleness resistance of the chain steel.

CN Patent Literature CN104532143A (published on April 22, 2015, entitled "Large-Size, High-Strength Mining Chain Steel and Manufacturing Method therefor") discloses an improved large-size mining chain steel with a diameter of 40-100 mm, a yield strength of ≥ 980 MPa, a tensile strength of ≥ 1180 MPa, an elongation of ≥ 13%, a reduction of area of ≥ 50% and a Charpy impact energy at room temperature of >100 J.

In addition, there are some technologies for optimizing steel based on the composition of 54 steel. For example, CN Patent Literature CN111101078A (published on May 5, 2020, entitled "Nickel-Free High-Strength Steel for Mining Round Link Chains and Manufacturing Method therefor") discloses a nickel-free high-strength steel for mining round link chains. By reducing the content of the precious metal element Ni and increasing the contents of alloying elements C, Si, Cr and Mo, it greatly reduces the production cost on the premise of ensuring mechanical properties.

By referring to the above prior art and other numerous existing improvement schemes, it is not difficult to find that researchers in this field mainly prepare high-strength steel for mining chains through optimized composition design, so as to improve the strength and wear resistance of mining chains made of such steel and extend their service life.

However, it should be noted that, in practical applications, the underground coal mines are typically humid working environments, and the high-strength mining chains are inevitably affected by environmental corrosion during service. Furthermore, the high-strength mining chains bear high stress and are quite sensitive to stress corrosion, which is prone to cause corrosion fatigue fracture during service (frequent low-load brittle fracture may occur in a few days or up to months), thus leading to the premature failure of the mining chains.

Therefore, the present disclosure aims to obtain a new mining chain steel with excellent comprehensive properties: it not only has high strength and can achieve good high strength and high toughness at a low alloy cost, but also demonstrates excellent corrosion resistance after coating or plating treatment to obtain chains, effectively solving the problem that the service life of existing mining chains is impaired due to the mismatch of strength and corrosion resistance.

### SUMMARY

Aiming at the problem in the prior art that the service life of existing mining chains is impaired due to the mismatch of strength and corrosion resistance, the objective of the present disclosure is to provide a high-strength chain steel, a high-corrosion-resistance mining chain and a manufacturing method therefor. While the addition amount of precious alloy elements in the high-strength chain steel is reduced, a chain made from the high-strength chain steel through a specific coating process not only has excellent comprehensive properties such as high strength and high toughness, but also has good corrosion resistance, and can be widely applied in environments with a large amount of corrosive medium, such as engineering machinery, mines, ships, and marine engineering.

To achieve the above objective, the present disclosure provides the following technical solutions:
The first aspect of the present disclosure provides a chain steel, comprising the following chemical elements in mass percentage: C: 0.20-0.30%, Si: 0.05-0.6%, preferably 0.15-0.6%, Mn: 1.0-1.8%, Cr: 0.4-0.8%, Ni: 0.6-1.2%, Mo: 0.5-0.9%, Ti: 0.01-0.03%, Al: 0.02-0.05%, B: 0.001-0.005%, N: 0.002-0.006%, and the balance being Fe and inevitable impurities.

Preferably, the chain steel has a chemical composition satisfying the following relational expression: 30000*B/(300*B+0.7*Ni+2*Cr+5*Mo) ≥ 6, more preferably 6 ≤ 30000*B/(300*B+0.7*Ni+2*Cr+5*Mo) ≤ 24.43, wherein element symbols respectively represent the numerical values preceding the % symbol of the mass percentage contents of corresponding elements.

Preferably, the inevitable impurities comprise P≤ 0.015%, S≤ 0.01%, and O≤ 0.002%.

Preferably, the chain steel has a microstructure of acicular martensite.

Preferably, the chain steel has the following properties: a yield strength Rp_{0.2} of ≥ 1050 MPa, a tensile strength Rₘ of ≥ 1200 MPa, an elongation A of ≥ 14%, a reduction of area Z of ≥ 50%, and a Charpy impact energy Akv at -20 °C of ≥ 60 J.

The second aspect of the present disclosure provides a chain, comprising: the chain steel described above and a zinc coating coated on the chain steel.

Preferably, the zinc coating of the chain has a thickness of 10-150 µm, more preferably 40-150 µm.

Preferably, the chain steel of the chain has a microstructure of tempered martensite and carbides dispersed interlamellarly.

Preferably, the chain has the following properties: a yield strength Rp_{0.2} of ≥ 1050 MPa, a tensile strength Rₘ of ≥ 1200 MPa, an elongation A of ≥ 14%, a reduction of area Z of ≥ 50%, a Charpy impact energy Akv at -20 °C of ≥ 60 J; and a corrosion rate of ≤ 0.2 g/m²·h after 120 h of 5% NaCl neutral salt spray corrosion test.

The third aspect of the present disclosure provides a method for manufacturing the chain described above, comprising the following steps performed sequentially:
S1, smelting and casting molten steel to obtain a cast slab;
S2, heating and rolling the cast slab, wherein the reduction ratio of the cast slab is ≥ 10;
S3, forming rings and welding;
S4, performing quenching heat treatment, wherein for the quenching heat treatment, a heating temperature is 840-980 °C, preferably 850-950 °C, and a holding time is 1-4 hours, preferably 1-3 hours, followed by water cooling for quenching;
S5, performing pickling pretreatment to obtain the chain steel;
S6, hot-dip galvanizing, wherein the chain steel after pickling pretreatment is subjected to preheating treatment followed by hot-dip galvanizing to obtain the chain comprising the chain steel and a zinc coating formed on the chain steel, wherein the temperature difference between the preheating temperature and the temperature of zinc bath used in the hot-dip galvanizing is -30 to 30 °C.

Preferably, in step S1, the smelting comprises electric furnace or converter smelting, LF refining, and VD or RH vacuum treatment; the casting adopts a continuous casting process.

Preferably, the VD or RH vacuum treatment is performed for 10-20 min; during casting, the superheat degree of the molten steel in the tundish is controlled to 15-40 °C.

Preferably, in step S2, during heating and rolling, the cast slab is heated at a heating temperature of ≥ 1150 °C for a heating time of 3-6 h, and a finishing rolling temperature is ≥ 850 °C; after rolling, air cooling or slow cooling is performed.

Preferably, in step S6, the preheating temperature is 400-550 °C, and the preheating time is ≥ 0.5 h; the temperature of zinc bath used in the hot-dip galvanizing is 400-530 °C.

Preferably, the zinc coating has a thickness of 10-150 µm, preferably 40-150 µm.

Preferably, the chain steel of the chain obtained in step 6 has a microstructure of tempered martensite and carbides dispersed interlamellarly.

Preferably, the chain has the following properties: a yield strength Rp_{0.2} of ≥ 1050 MPa, a tensile strength Rₘ of ≥ 1200 MPa, an elongation A of ≥ 14%, a reduction of area Z of ≥ 50%, a Charpy impact energy Akv at -20 °C of ≥ 60 J; and a corrosion rate of less than 0.2 g/m²·h after 120 h of 5% NaCl neutral salt spray corrosion test.

The design principles of chemical elements in the high-strength chain steel according to the present disclosure are as follows. In the present disclosure, unless otherwise explicitly stated, element contents are expressed as a mass percentage.

C: C element is an essential element for ensuring the strength of the steel. Increasing the C content in the steel will enhance its capability for non-equilibrium microstructure transformation, thereby significantly improving its strength. In the present disclosure, the diffusion of C in the steel can be inhibited by quenching heat treatment to induce a shear-type martensite phase transformation, thus significantly improving the strength of the steel. However, the C content in the steel should not be excessively high. An overly high C content will adversely affect the plasticity and toughness of the steel, and will significantly increase the carbon equivalent of the steel, deteriorating the weldability of the steel. Therefore, in the high-strength chain steel according to the present disclosure, the mass percentage content of C is controlled to 0.20% - 0.30%.

Si: Si element can solid-dissolve in the steel and has a solid solution strengthening effect, significantly improving the yield strength, fatigue strength, and hardness of the steel. However, Si has very low solubility in cementite, thus the Si content in the steel should not be excessively high. An overly high Si content will not only lead to the formation of carbide-free bainite microstructure, but also increase the brittleness of the steel. Therefore, in the high-strength chain steel according to the present disclosure, the mass percentage content of Si is controlled to 0.05-0.6%, preferably 0.15-0.6%.

Mn: Mn element can improve the stability of austenite in the steel and also enhance the hardenability of the steel. Furthermore, Mn can also improve the strength of martensite in the steel through solid solution strengthening, thereby increasing the strength of the steel. However, it should be noted that the Mn content in the steel should not be excessively high. An overly high Mn content will cause austenite grains to tend to grow and promote the segregation of harmful elements at grain boundaries during quenching heating. Therefore, in the high-strength chain steel according to the present disclosure, the mass percentage content of Mn is controlled to 1.0-1.8%.

Cr: The addition of an appropriate amount of Cr element can improve the hardenability of the steel and has a secondary hardening effect, which enables the formation of a hardened martensite microstructure and is conducive to enhancing the strength of the steel. In addition, Cr carbides can slow down the grain growth in the heat-affected zone at the weld joint, which is very beneficial to the welding of steel. The addition of appropriate amounts of Cr and Ni to steel is beneficial for improving the corrosion resistance of steel. However, the Cr content in the steel should not be excessively high. If the Cr content in the steel is excessively high, a large amount of carbides will be generated and accumulate at the grain boundaries, reducing the toughness of the steel and significantly increasing the carbon equivalent, thus deteriorating the weldability of the high-strength steel. Therefore, in the high-strength chain steel according to the present disclosure, the mass percentage content of Cr is controlled to 0.4-0.8%.

Ni: Ni element is one of the main strengthening elements and can be present in the steel in the form of solid solution and is infinitely soluble with iron. When Ni is used in combination with Cr, the hardenability of the steel will be significantly improved. Furthermore, the addition of an appropriate amount of Ni to the steel can lower the C content at the eutectoid point, strengthen ferrite, and refine and increase pearlite, thereby improving the strength of the steel without significantly affecting its plasticity. Ni can improve the fatigue resistance of the steel, reduce its sensitivity to notch, lower its ductile-to-brittle transition temperature at low temperature, and improve its impact toughness. However, Ni is a precious alloying element, and the addition of a large amount of Ni will lead to an increase in alloy cost. Therefore, in the high-strength chain steel according to the present disclosure, the mass percentage content of Ni element is controlled to 0.6-1.2%.

Mo: Mo element mainly exists in the steel in solid solution form and has a solid solution strengthening effect, which is beneficial to improving the hardenability of the steel, enabling the formation of martensite in the steel during quenching. However, the Mo content in the steel should not be excessively high. When the Mo content in the steel is excessively high, the carbon equivalent of the steel will be significantly increased, which is detrimental to the weldability of the steel. In addition, Mo is also a precious alloying element, and the addition of a large amount of Mo will lead to an increase in alloy cost. Therefore, in the high-strength chain steel according to the present disclosure, the mass percentage content of Mo is controlled to 0.5-0.9%.

Ti: Ti element has a strong affinity for nitrogen, oxygen and carbon with a high precipitation temperature, which makes it an effective element for fixing nitrogen and carbon in the steel and enables the formation of fine precipitated phases in the steel, thereby improving the strength and toughness of the steel, especially the impact toughness at low temperatures. However, an excessively high Ti content in the steel will lead to the formation of coarse angular TiN particles during smelting, reducing the impact toughness of the steel. Therefore, the Ti content is controlled to 0.01-0.03% in the high-strength chain steel according to the present disclosure.

Al: Al element mainly functions for deoxidation and nitrogen fixation. AlN, formed by the combination of Al and N, can effectively refine the grains. However, it should be noted that the Al content in the steel should not be excessively high. An overly high Al content in the steel will affect the casting performance of the steel and impair its toughness. Therefore, in the high-strength chain steel according to the present disclosure, the mass percentage content of Al is controlled to 0.02% - 0.05%.

B: B mainly functions to enhance the hardenability of the steel and improve the strength of the steel after quenching and tempering, while slightly increasing its plasticity, thus saving other rare and precious metals such as nickel, chromium and molybdenum. However, B is a highly reactive element with a strong affinity for oxygen, nitrogen and other elements, readily forming boron oxide, boron nitride and other compounds. This leads to the inactivation of B and an increase of the hardenability fluctuation of the steel, impairing stability of steel properties. In addition, boron is a reactive and segregation-prone element that tends to segregate at grain boundaries and may induce temper brittleness, which is detrimental to the toughness of the steel. Therefore, the content of B is controlled to 0.001-0.005% in the high-strength chain steel according to the present disclosure.

N: N is an austenite-forming element and also an MX-type precipitate-forming element, and thus functions to refine grains. However, in boron-containing steel, N in the steel will combine with B, thereby causing B in the steel to lose its alloying effect. To prevent the N element from consuming the B element, the content of N in the steel must be strictly controlled. Therefore, the mass percentage content of N is controlled to 0.002-0.006% in the high-strength chain steel according to the present disclosure.

By virtue of the rational design of main alloying elements, the present disclosure improves the hardenability and mechanical properties of the steel and reduces the addition of precious alloy elements by adding B, and enables the high-strength chain steel according to the present disclosure to have excellent comprehensive properties by taking full advantage of the effects of various alloying elements and their interactions on the microstructure and mechanical properties.

In a preferred embodiment, in the chemical composition of the chain steel, the contents of B, Cr, Ni and Mo satisfy the following relational expression: 30000*B/(300*B+0.7*Ni+2*Cr+5*Mo) ≥ 6, more preferably 6 ≤ 30000*B/(300*B+0.7*Ni+2*Cr+5*Mo) ≤ 24.43, wherein element symbols respectively represent the numerical values preceding the % symbol of the mass percentage contents of corresponding elements.

In the high-strength chain steel according to the present disclosure, Cr, Ni and Mo are important alloying elements, each contributing differently to the strength, toughness and hardenability of the chain steel. However, the excessive addition of these precious alloying elements will substantially increase the cost of the steel. Therefore, an appropriate amount of Cr, Ni and Mo is added to the chain steel according to the present disclosure to interact with the trace amount of B added thereto. When the content of B and the contents of Cr, Ni and Mo satisfies the relational expression 30000*B/(300*B+0.7*Ni+2*Cr+5*Mo) ≥ 6, the B element can solid-dissolve in the matrix and segregate at the austenite grain boundaries, which improves the stability of austenite and increases the hardenability of the steel during the heat treatment processes in the chain manufacturing, thereby enabling the steel to have excellent comprehensive properties such as high strength and high toughness. When the relational expression among the contents of B, Cr, Ni and Mo (expressed as 30000*B/(300*B+0.7*Ni+2*Cr+5*Mo)) is <6, the content of B added to the steel is too low to enhance the hardenability of the steel. In such case, precious alloying elements have to be added to ensure that the chain steel achieves good high strength and high toughness during quenching heat treatment and hot-dip galvanizing, which increases the production cost of the chain.

In the chain steel according to the present disclosure, the inevitable impurities are required to satisfy P ≤ 0.015%, S ≤ 0.01%, O ≤ 0.002%. P, S, and O are all impurity elements in the steel. Where technical conditions permit, the content of impurity elements in the steel should be reduced as much as possible to obtain the chain steel with better performance and higher quality. In the chain steel according to the present disclosure, P and S are both inevitable harmful impurity elements in the steel, and both will deteriorate the properties of the steel. Although P can improve the weather resistance of the steel, its side effects are more significant overall. Therefore, in the present disclosure, P is controlled to ≤ 0.015%, S is controlled to ≤ 0.01%. Furthermore, in the present disclosure, the impurity element O can form oxides and composite inclusions with deoxidizing elements such as Ti, B, and Al in the steel, which is detrimental to the properties of the steel. Therefore, in the present disclosure, O is controlled to ≤ 0.002%.

Of course, in some other embodiments, other harmful elements such as As, Pb, Sn, Sb, Bi and the like may also be present in the steel. While in compliance with the requirements of national laws, regulations, and standards, the contents of these harmful elements should be reduced as much as possible.

Compared with existing production technologies, the present disclosure has the following beneficial effects:
1. The present disclosure adopts a rational chemical composition design combined with an optimized manufacturing method. The present disclosure improves the hardenability and mechanical properties of the steel and reduces the addition amount of precious alloying elements by adding B, and enables the chain steel according to the present disclosure to have excellent comprehensive properties by taking full advantage of the effects of various alloying elements and their interactions on the microstructure and mechanical properties. Manufacturing the chain by subjecting the chain steel to online quenching and hot-dip galvanizing treatment allows for, on the one hand, the precipitation of fine dispersed carbides in the supersaturated solid solution formed in the chain steel after quenching heat treatment, which improves the properties of the chain steel, on the other hand, the formation of a zinc coating (or galvanized coating) with a certain thickness on the surface of the chain steel, thereby enabling the chain to have excellent corrosion resistance.
2. After the zinc coating is applied to the surface of the chain steel according to the present disclosure, it can isolate the corrosive medium from contacting the chain steel, thereby improving the corrosion resistance of the chain. When the zinc coating on partial areas of the chain wears off, the zinc coating on the remaining areas can still provide cathodic protection to prevent corrosion from occurring during the service of the chain, thus increasing the service life of the chain.
3. The high-strength chain steel according to the present disclosure has a rational chemical composition and process design, along with a wide process window, enabling mass commercial production.
4. The high-strength chain steel and chain according to the present disclosure achieve excellent high strength and toughness as well as good corrosion resistance at a low cost, and can be fabricated into high-strength and corrosion-resistant structural components, as well as various high-performance industrial chains such as mining and mooring chains, and is widely applied in engineering machinery, mines, marine engineering and other scenarios requiring steel with high strength, high toughness and high corrosion resistance.
5. The high-corrosion-resistance mining chain made of the chain steel according to the present disclosure not only have high strength, toughness and plasticity, but also exhibit excellent corrosion resistance, thus having broad application prospects.

### DETAILED DESCRIPTION

To facilitate a better understanding of the aforementioned technical solutions according to the present disclosure, the technical solutions of the present disclosure are further described below with reference to the Examples.

The present disclosure provides a high-strength chain steel, comprising the following chemical elements in mass percentage: C: 0.20-0.30%, Si: 0.05-0.6%, preferably 0.15-0.6%, Mn: 1.0-1.8%, Cr: 0.4-0.8%, Ni: 0.6-1.2%, Mo: 0.5-0.9%, Ti: 0.01-0.03%, Al: 0.02-0.05%, B: 0.001-0.005%, N: 0.002-0.006%, and the balance being Fe and inevitable impurities.

By virtue of the rational design of main alloying elements, the present disclosure improves the properties of the steel and reduces the addition of precious alloy elements by adding B, and precisely control the microstructure of the steel according to the present disclosure by taking full advantage of the effects of various alloying elements and their interactions on the microstructure and mechanical properties, to ensure that when the chain steel according to the present disclosure is made into the chain via hot-dip galvanizing, a mixed microstructure of tempered martensite + carbides dispersed interlamellarly is formed in the chain steel. This microstructure endows the chain according to the present disclosure with both high strength and toughness-plasticity matching, as well as good wear resistance and fatigue resistance.

In a specific embodiment, the chain steel has a chemical composition satisfying the following relational expression: 30000*B/(300*B+0.7*Ni+2*Cr+5*Mo)≥ 6, more preferably 6 ≤ 30000*B/(300*B+0.7*Ni+2*Cr+5*Mo) ≤ 24.43, wherein element symbols respectively represent the numerical values preceding the % symbol of the mass percentage contents of corresponding elements.

In the present disclosure, Cr, Ni and Mo are important alloying elements, each contributing differently to the strength, toughness and hardenability of the high-strength chain steel. However, the excessive addition of precious alloying elements will substantially increase the cost of the steel. Therefore, an appropriate amount of Cr, Ni and Mo is added to the chain steel according to the present disclosure to interact with the trace amount of B added thereto. When the content of B and the contents of Cr, Ni and Mo satisfies the relational expression 30000*B/(300*B+0.7*Ni+2*Cr+5*Mo) ≥ 6, the B element can solid-dissolve in the matrix and segregate at the austenite grain boundaries, which improves the stability of austenite and increases the hardenability of the steel during the heat treatment processes in the chain manufacturing, thereby enabling the steel to have excellent comprehensive properties such as high strength and high toughness. When 30000*B/(300*B+0.7*Ni+2*Cr+5*Mo)< 6, the content of B added to the steel is too low to enhance the hardenability of the steel; therefore, precious alloying elements have to be added to ensure that the chain steel achieves good high strength and high toughness during quenching and hot-dip galvanizing, which increases the production cost of the chain.

In the present disclosure, P, S, and O are all impurity elements in the steel. Where technical conditions permit, the content of impurity elements in the steel should be reduced as much as possible to obtain the chain steel with better performance and higher quality. P and S are both inevitable harmful impurity elements in the steel, and both will deteriorate the properties of the steel. Although P can improve the weather resistance of the steel, its side effects are more significant overall. Therefore, among the inevitable impurities, P ≤ 0.015%, S ≤ 0.01%. Furthermore, the impurity element O can form oxides and composite inclusions with deoxidizing elements such as Ti, B, and Al in the steel, which is detrimental to the properties of the steel. Therefore, O ≤ 0.002%.

In a specific embodiment, the chain steel has a microstructure of acicular martensite. The chain steel in the chain formed after subjecting this high-strength chain steel to quenching heat treatment and hot-dip galvanizing has a microstructure of tempered martensite and carbides dispersed interlamellarly.

The high-strength mining chain steel has the following properties: a yield strength Rp_{0.2} of ≥ 1050 MPa, a tensile strength Rₘ of ≥ 1200 MPa, an elongation A of ≥ 14%, a reduction of area Z of ≥ 50%, and a Charpy impact energy Akv at -20 °C of ≥ 60 J.

The chain manufactured via hot-dip galvanizing the surface of the chain steel has a corrosion rate of ≤ 0.2 g/m²·h after 120 h of 5% NaCl neutral salt spray corrosion test.

The present disclosure provides a chain manufactured with the above-mentioned chain steel, and the chain has the following properties: a yield strength Rp_{0.2} of ≥ 1050 MPa, a tensile strength Rₘ of ≥ 1200 MPa, an elongation A of ≥ 14%, a reduction of area Z of ≥ 50%, a Charpy impact energy Akv at -20 °C of ≥ 60 J, and a corrosion rate of ≤ 0.2 g/m²·h after 120 h of 5% NaCl neutral salt spray corrosion test.

The present disclosure further provides a method for manufacturing the above-mentioned high-corrosion-resistance mining chain, which has a simple production process, and the obtained chain has excellent high strength and toughness as well as good corrosion resistance.

The method for manufacturing the chain steel and chain according to the present disclosure specifically includes the following steps:
S1, Smelting and casting molten steel to obtain a cast slab.

Specifically, the smelting operation includes electric furnace or converter smelting, LF refining, and VD or RH vacuum treatment. That is to say, smelting is performed using an electric furnace or converter, followed by LF refining and VD or RH vacuum treatment, wherein the vacuum treatment is performed for 10-20 minutes, and the molten steel is tapped for casting after the chemical composition meets the requirements of the chain steel. Then, during casting process, the molten steel is cast into a slab using continuous casting, controlling the superheat degree of the molten steel in the tundish to 15-40°C, and a cast slab with a chemical composition that meets the requirements of the chain steel is ultimately obtained.

S2, Heating and rolling the cast slab, wherein the reduction ratio of the cast slab is ≥ 10.

Specifically, the cast slab is heated in a heating furnace, then tapped, subsequently subjected to high-pressure water descaling, and then subjected to rolling to roll the cast slab into round steel of finished size; wherein the cast slab is controlled to be heated at a heating temperature of ≥ 1150 °C for a heating time of 3-6 h, and a finishing rolling temperature is ≥ 850 °C. After rolling, air cooling or slow cooling is performed to room temperature. The reduction ratio of the cast slab is controlled to ≥ 10 during rolling. The resulting round steel has a finished size specification of Φ 30 to 150 mm.

S3, Forming rings and welding. The round steel is cut to fixed length, then formed into individual rings on a chain making machine, and then weld them into complete rings by flash welding to obtain a chain-like substrate.

S4, Performing quenching heat treatment, wherein for the quenching heat treatment, a heating temperature is 850-950 °C, and a holding time is 1-3 hours, followed by water cooling for quenching.

Specifically, the chain-like substrate obtained after forming rings and welding is subjected to quenching heat treatment at a heating temperature of 850-950 °C for a heating time of 1-3 hours, followed by water cooling for quenching. After high-temperature heating, fine austenite grains are formed in the chain-like substrate, with an austenite grain size of ≥ Grade 7. After quenching, the microstructure of the chain-like substrate transforms from the austenite microstructure under high temperature to a fine acicular martensite microstructure.

S5, Pickling pretreatment. The chain-like substrate after quenching heat treatment is subjected to pickling pretreatment to remove the oxide scale on the surface of the chain-like substrate after quenching, obtaining the chain steel. Preferably, a layer of flux is applied to the surface of the chain steel to maintain a certain level of activity on the chain steel surface after being subjected to pickling pretreatment, preventing oxidation of the chain steel during subsequent preheating treatment and enhancing the bonding force between the zinc coating and the chain steel. It should be noted that the flux used in the present disclosure is a commonly used auxiliary agent in galvanizing in the art, which are commercially available.

S6, Hot-dip galvanizing. The chain steel after pickling pretreatment is subjected to preheating treatment followed by hot-dip galvanizing to obtain a chain comprising the chain steel and a zinc coating formed on the surface of the chain steel, wherein the temperature difference between the preheating temperature for the preheating treatment and the temperature of zinc bath used in hot-dip galvanizing is controlled to -30 to 30°C.

Specifically, the chain steel is subjected to preheating treatment before hot-dip galvanizing to prevent problems such as zinc explosion (or zinc spattering) during hot-dip galvanizing process, thereby obtaining a high-corrosion-resistance mining chain. The temperature difference between the preheating temperature of the chain and the temperature of zinc bath used in hot-dip galvanizing is controlled to -30 to 30°C; wherein the preheating temperature is 400 - 550°C, and the preheating time is ≥ 0.5 h; the temperature of zinc bath used in hot-dip galvanizing is 400 - 530 °C. The thickness of the zinc coating on the surface of the chain steel is controlled to 10 - 150 µm, preferably 40 - 150 µm.

During hot-dip galvanizing, fine carbides precipitate from the supersaturated acicular martensite microstructure formed after quenching of the chain steel. While this results in a partial decrease in the strength of the chain steel, its elongation and impact toughness are improved. The fine acicular martensite microstructure facilitates the precipitation of fine, dispersed carbides in the chain steel during hot-dip galvanizing, thereby obtaining a chain with excellent strength and toughness.

The chain steel in the high-corrosion-resistance mining chain described above has a microstructure of tempered martensite and carbides dispersed interlamellarly.

The high-corrosion-resistance mining chain described above has the following properties: a yield strength Rp_{0.2} of ≥ 1050 MPa, a tensile strength Rₘ of ≥ 1200 MPa, an elongation A of ≥ 14%, a reduction of area Z of ≥ 50%, a Charpy impact energy Akv at -20 °C of ≥ 60 J; and a corrosion rate of less than 0.2 g/m²·h after 120 h of 5% NaCl neutral salt spray corrosion test.

The present disclosure, by virtue of rational design of alloying elements combined with optimized manufacturing process and taking full advantage of the effects of various alloying elements and the manufacturing process of the chain steel and chain on the microstructure, precisely controls the microstructure of the chain steel. An acicular martensite microstructure is formed in the chain steel obtained after quenching heat treatment. The subsequent hot-dip galvanizing treatment of the chain steel allows for, on the one hand, the precipitation of fine, dispersed carbides in the chain steel during hot-dip galvanizing, thus improving the strength and toughness of the chain, on the other hand, the formation of a zinc coating with a certain thickness on the surface of the chain steel, thereby improving the corrosion resistance of the chain.

In the manufacturing process of the chain according to the present disclosure, the conventional quenching process of chain is combined with the hot-dip galvanizing process, and the tempering process of chain is omitted. By fully utilizing the precipitation of carbides in the steel during hot-dip galvanizing process, the efficient production of the high-strength corrosion-resistance chain is achieved. As a result, the high-strength chain has both high strength and toughness-plasticity matching, as well as good corrosion resistance.

The high-strength chain steel, high-corrosion-resistance mining chain and manufacturing method therefor according to the present disclosure are further described below reference to the specific examples. It should be clearly stated that the following examples are only used to describe the specific embodiments of the present disclosure and do not constitute any limitation on the protection scope of the present disclosure.

### EXAMPLES

### Examples 1-6

As shown in Tables 1, 2-1, and 2-2, the high-strength chain steels and high-corrosion-resistance mining chains of Examples 1-6 are manufactured by the following steps:
(1) Smelting and continuous casting were performed in accordance with the chemical composition shown in Table 1 below to obtain cast slabs. Smelting could be performed in an electric furnace or converter, followed by LF refining and VD or RH vacuum treatment. The vacuum treatment was performed for 10-20 min, and the molten steel was tapped after the chemical composition met the requirements. Then, the molten steel could be cast into cast slabs using continuous casting. The superheat degree of the molten steel in the tundish was controlled to 15-40 °C during continuous casting.
(2) Heating and rolling: The cast slabs were heated in a heating furnace, then subjected to high-pressure water descaling, and subsequently rolled to obtain round steels of finished size. The rolled round steels had a finished size specification of Φ 30 to 150 mm, and the reduction ratio of the cast slabs was controlled to ≥ 10. During rolling, the cast slabs after being heated were rolled to finished size, wherein the cast slabs were controlled to be heated at the heating temperature of ≥ 1150 °C for a heating time of 3-6 h, and the finishing rolling temperature was ≥ 850 °C. After rolling, air cooling or slow cooling was performed to room temperature.
(3) Forming rings and welding: The round steels were cut to fixed length and formed into individual rings on a chain making machine, subsequently welded them into chain-like substrates of complete rings by flash welding.
(4) Quenching heat treatment: the chain-like substrates obtained after forming rings and welding were subjected to quenching heat treatment. For the quenching heat treatment, the heating temperature was controlled to 840-980 °C and the holding time was 1-4 hours, followed by water cooling for quenching.
(5) Pickling pretreatment: The chain-like substrates after quenching were subjected to pickling pretreatment to remove the oxide scale on the surfaces of the chain-like substrates. Then, the chain-like substrates after pickling pretreatment were subjected to preheating treatment. In order to prevent problems such as zinc explosion (or zinc spattering) during subsequent hot-dip galvanizing, the chain-like substrates after pickling pretreatment were subjected to preheating treatment at the preheating temperature of 400-550 °C for ≥ a preheating time of 0.5 h. For the chain-like substrate after pickling pretreatment, the temperature difference between the preheating temperature and the temperature of zinc bath used in the subsequent hot-dip galvanizing was -30 to 30°C.
(6) Hot-dip galvanizing: The chain-like substrates after pickling pretreatment and preheating treatment were hot-dip galvanized at a zinc bath temperature of 400-530 °C, and the thickness of the zinc coating on the chain steel surface was controlled to 10-150 µm. High-corrosion-resistance mining chains comprising chain steel and a zinc coating on the chain steel surface were obtained.

The chemical composition designs and related process parameters of the high-strength chain steels and high-corrosion-resistance mining chains of Examples 1-6 all met the design requirements of the present disclosure.

### Comparative Examples 1-2

The comparative steels of Comparative Examples 1-2 were finished steels from different manufacturers, and their chemical compositions are shown in Table 1 below. The manufacturing processes of the comparative steels differed from those of Examples 1-6, the heat treatment processes adopted for the comparative steels of Comparative Examples 1-2 referred to the parameters recommended by the manufacturers, with the specific values shown in Tables 2-1 and 2-2. The tempering temperature and tempering time in Table 2-2 all represent the tempering process of Comparative Examples 1-2.

Table 1 shows the chemical compositions of the chain steels of Examples 1-6 and the comparative steels of Comparative Examples 1-2.

**Table 1 (wt.%, the balance being Fe and other impurities in addition to P and S)**

| | C | Si | Mn | P | S | Cr | Ni | Mo | Ti | Al | B | N | O | 30000B/(300B+0. 7Ni+2Cr+5Mo) |
|---|---|---|---|---|---|---|---|---|---|---|---|---|---|---|
| Example 1 | 0.25 | 0.34 | 1.55 | 0.01 | 0.007 | 0.55 | 0.78 | 0.81 | 0.01 6 | 0.021 | 0.0013 | 0.0035 | 0.0016 | 6.41 |
| Example 2 | 0.28 | 0.47 | 1.69 | 0.015 | 0.008 | 0.41 | 0.63 | 0.88 | 0.02 8 | 0.035 | 0.0031 | 0.0047 | 0.0013 | 14.11 |
| Example 3 | 0.22 | 0.07 | 1.39 | 0.006 | 0.01 | 0.79 | 0.89 | 0.68 | 0.02 9 | 0.048 | 0.0018 | 0.0059 | 0.0019 | 8.79 |
| Example 4 | 0.3 | 0.57 | 1.06 | 0.013 | 0.009 | 0.65 | 0.95 | 0.72 | 0.02 4 | 0.026 | 0.0028 | 0.0042 | 0.0020 | 13.11 |
| Example 5 | 0.24 | 0.25 | 1.22 | 0.01 | 0.002 | 0.56 | 1.18 | 0.52 | 0.01 2 | 0.032 | 0.0049 | 0.0023 | 0.0010 | 24.43 |
| Example 6 | 0.21 | 0.15 | 1.74 | 0.012 | 0.002 | 0.62 | 1.02 | 0.63 | 0.02 4 | 0.041 | 0.0041 | 0.0056 | 0.0014 | 19.42 |
| Comparativ e Example 1 | 0.23 | 0.15 | 1.2 | 0.008 | 0.006 | 0.55 | 0.98 | 0.51 | 0.00 1 | 0.027 | 0.0005 | 0.0086 | 0.0012 | 3.34 |
| Comparativ e Example 2 | 0.21 | 0.25 | 1.25 | 0.013 | 0.006 | 1.5 | 1.0 | 0.35 | 0.00 2 | 0.03 | 0.0003 | 0.01 | 0.0019 | 1.62 |

Tables 2-1 shows the specific process parameters for the preparation of the finished chains of Examples 1-6 and the comparative chains of Comparative Examples 1-2.

**Table 2-1**

| Number | Step (1) | | | Step (2) | | | Round steel specification (mm) |
|---|---|---|---|---|---|---|---|
| | Smelting and casting | Vacuum treatment time (min) | Superheat degree of molten steel (°C) | Heating temperature (°C) | Heating time (h) | Finishing rolling temperature (°C) | |
| Example 1 | Electric furnace + LF + VD + Continuous casting | 15 | 23 | 1220 | 4 | 960 | Φ125 |
| Example 2 | Electric furnace + LF + VD + Continuous casting | 12 | 18 | 1200 | 5 | 880 | Φ30 |
| Example 3 | Electric furnace + LF + VD + Continuous casting | 18 | 35 | 1150 | 3 | 920 | Φ48 |
| Example 4 | Electric furnace + LF + RH + Continuous casting | 20 | 25 | 1240 | 4 | 900 | Φ60 |
| Example 5 | Electric furnace + LF + RH + Continuous casting | 14 | 30 | 1180 | 6 | 850 | Φ100 |
| Example 6 | Electric furnace + LF + RH + Continuous casting | 13 | 39 | 1220 | 4 | 980 | Φ150 |
| Comparative Example 1 | Electric furnace + LF + VD + Continuous casting | | | | | | Φ48 |
| Comparative Example 2 | Electric furnace + LF + RH + Continuous casting | | | | | | Φ38 |

Tables 2-2 shows the specific process parameters for the preparation of the finished chains of Examples 1-6 and the comparative chains of Comparative Examples 1-2.

**Table 2-2**

| No. | Step (4) | | Step (5) | | Step (6) | |
|---|---|---|---|---|---|---|
| | Quenching temperature (°C) | Holding time (h) | Preheating/ Tempering temperature (°C) | Preheating/ Tempering time (h) | Zinc bath temperature (°C) | Zinc coating thickness (µm) |
| Example 1 | 980 | 3 | 510 | 1.5 | 500 | 125 |
| Example 2 | 880 | 1 | 430 | 0.5 | 410 | 15 |
| Example 3 | 930 | 2 | 415 | 0.8 | 435 | 80 |
| Example 4 | 910 | 2 | 470 | 1.2 | 450 | 40 |
| Example 5 | 840 | 3 | 490 | 1.5 | 470 | 105 |
| Example 6 | 950 | 4 | 540 | 2 | 530 | 145 |
| Comparative Example 1 | 880 | 1 | 410 | 1 | | |
| Comparative Example 2 | 880 | 1 | 430 | 1 | | |

Finished chains prepared in Examples 1-6 and comparative chains of Comparative Examples 1-2 were collected, and their properties were further tested to obtain the properties of the finished chains of each Example and Comparative Example.

In the present disclosure, neutral salt spray corrosion test, tensile test and impact property test were conducted on the finished chains of Examples 1-6 and the comparative chains of Comparative Examples 1-2 respectively, and the test results are listed in Table 3.

The specific testing methods for the aforementioned neutral salt spray corrosion test, tensile test and impact test are as follows:
Neutral salt spray corrosion test was conducted through the following steps: 100 mm-long round steels were taken from the finished chains of Examples 1-6 and the comparative chains of Comparative Examples 1-2 as salt spray corrosion test specimens, with both end surfaces sealed with silicone rubber. 5 wt% NaCl salt spray corrosion tests were performed in accordance with the standard GB/T 10125 (test chamber temperature: 35 °C, saturation barrel temperature: 47 °C, corrosive medium: 5 wt% NaCl aqueous solution, pH=6.5, the test specimens were positioned at a 20° angle to the vertical direction, the test was performed for 120 h with a continuous spraying mode, and the salt spray deposition rate was 1.5 mL/(h·80 cm²)). After 120 h of neutral salt spray test, the test specimens were taken out, the silicone rubber at both ends was stripped off, surface corrosion products were removed, and the specimens were blow-dried and weighed to record the mass as *M'*. The salt spray corrosion rate *R* of the test specimens of each Example and Comparative Example was then calculated using: $R = \left(M-M′\right) / \left(S⋅T\right) ,$ wherein *M* is the initial mass of the specimen in the unit of grams (g); *M'* is the mass of the specimen after removing corrosion products and blow-drying in the unit of grams (g); *S* is the corrosion test area of the specimen in the unit of square meters (m²); *T* is the corrosion time in the unit of hours (h); the salt spray corrosion rate *R* is in the unit of g/m²·h.

Tensile test: The finished chains of Examples 1-6 and the comparative chains of Examples 1-2 were sampled and prepared into tensile test specimens in accordance with the national standard GB/T 2975, and tensile property tests were conducted in accordance with the national standard GB/T 228.1 to determine the yield strength Rp_{0.2}, tensile strength Rₘ, elongation A and reduction of area Z of the finished chains of Examples 1-6 and the comparative chains of Comparative Examples 1-2.

Impact test: The finished chains of Examples 1-6 and the comparative chains of Examples 1-2 were sampled and prepared into impact test specimens according to national standard GB/T 2975, and impact property tests were conducted in accordance with the national standard GB/T 229 to determine the Charpy impact energy Akv at low temperature of the coated finished chains of Examples 1-6 and the chains of Comparative Examples 1-2.

Table 3 shows the property parameters of the finished chains of Examples 1-6 and the comparative chains of Comparative Examples 1-2.

**Table 3**

| | Yield strength R_{p0.2} (MPa) | Tensile strength Rₘ (MPa) | Elongation A (%) | Reduction of area Z (%) | Charpy impact energy Aₖᵥ at -20 °C (J) | Salt spray corrosion rate (g/m²·h) |
|---|---|---|---|---|---|---|
| Example 1 | 1160 | 1278 | **15** | 57 | **69** | 0.17 |
| Example 2 | **1185** | **1315** | 15.5 | **55** | 100 | 0.15 |
| Example 3 | 1127 | 1281 | 17.5 | 65 | 89 | **0.19** |
| Example 4 | 1085 | **1212** | 17 | 61 | 95 | 0.12 |
| Example 5 | 1105 | 1256 | 18.5 | 68 | 79 | 0.13 |
| Example 6 | **1076** | 1225 | 18 | 65 | 96 | 0.11 |
| Comparative Example 1 | 1104 | 1289 | 13 | 58 | 51 | 2.61 |
| Comparative Example 2 | 975 | 1153 | 17 | 57 | 77 | 1.79 |

As shown in Table 3, the high-corrosion-resistance mining chains of the Examples 1-6 of the present disclosure exhibited excellent comprehensive properties, with a yield strength Rp_{0.2} of 1076 - 1185 MPa, a tensile strength Rₘ of 1212-1315 MPa, an elongation A of ≥ 14%, a reduction of area Z of ≥ 50%, and a Charpy impact energy Akv at -20 °C of ≥ 60 J. The neutral salt spray corrosion rate of the high-corrosion-resistance mining chains of Examples 1-6 was ≤ 0.19 g/m²·h, which was much lower than that of the comparative chains of Comparative Examples 1-2. It can be seen that the high-strength chain steel of the present disclosure after quenching heat treatment and hot-dip galvanizing exhibited significantly better corrosion resistance than that of the existing comparative chains selected in Comparative Examples 1-2.

In summary, the present disclosure adopts a rational chemical composition design, combines the conventional chain heat treatment with the subsequent galvanizing process to form an optimized quenching heat treatment and hot-dip galvanizing process, and ultimately obtains a high-corrosion-resistance mining chain with excellent properties. The chain steel according to the present disclosure has excellent comprehensive properties. The chain steel not only has high strength but also excellent toughness-plasticity matching, and the mining chain made of this chain steel has excellent corrosion resistance, effectively solving the problem that the service life of existing mining chains is impaired due to the mismatch of strength, toughness, plasticity and corrosion resistance. The chain steel can be fabricated into various high-performance industrial chains such as mining chains and mooring chains, which are widely applied in engineering machinery, mines, marine engineering and other scenarios requiring chains with high strength, high toughness and high corrosion resistance.

It should be noted that all the technical features described in the present disclosure can be freely combined in any ways unless contradicted with each other. Various modifications or variations may be made to the present disclosure without departing from the scope thereof. Such modifications or variations will be apparent to those skilled in the art. For example, a feature shown or described as part of one embodiment may be used with another embodiment to produce yet another embodiment. Therefore, the present disclosure is intended to cover such modifications and variations that fall within the scope of the appended claims and their equivalents.

## Claims

1. A chain steel, comprising the following chemical elements in mass percentage: C: 0.20-0.30%, Si: 0.05-0.6%, preferably 0.15-0.6%, Mn: 1.0-1.8%, Cr: 0.4-0.8%, Ni: 0.6-1.2%, Mo: 0.5-0.9%, Ti: 0.01-0.03%, Al: 0.02-0.05%, B: 0.001-0.005%, N: 0.002-0.006%, and the balance being Fe and inevitable impurities.

2. The chain steel according to claim 1, wherein the chain steel has a chemical composition satisfying the following relational expression: 30000*B/(300*B+0.7*Ni+2*Cr+5*Mo)≥ 6, preferably 6 ≤ 30000*B/(300*B+0.7*Ni+2*Cr+5*Mo) ≤ 24.43, wherein element symbols respectively represent the numerical values preceding the % symbol of the mass percentage contents of corresponding elements.

3. The chain steel according to claim 1, wherein the inevitable impurities comprise P, S, and O, wherein P ≤ 0.015%, S ≤ 0.01%, and O ≤ 0.002%.

4. The chain steel according to claim 1, wherein the chain steel has a microstructure of acicular martensite.

5. The chain steel according to claim 1, wherein the chain steel has the following properties: a yield strength Rp_{0.2} of ≥ 1050 MPa, a tensile strength Rₘ of ≥ 1200 MPa, an elongation A of ≥ 14%, a reduction of area Z of ≥ 50%, and a Charpy impact energy Aₖᵥ at -20 °Cof ≥ 60 J.

6. A chain comprising: the chain steel according to any one of claims 1 to 5, and a zinc coating coated on the chain steel.

7. The chain according to claim 6, wherein the zinc coating has a thickness of 10-150 µm, preferably 40-150 µm; and/or the chain steel has a microstructure of tempered martensite and carbides dispersed interlamellarly.

8. The chain according to claim 6, wherein the chain has the following properties: a yield strength Rp_{0.2} of ≥ 1050 MPa, a tensile strength Rₘ of ≥ 1200 MPa, an elongation A of ≥ 14%, a reduction of area Z of ≥ 50%, a Charpy impact energy Aₖᵥ at -20 °C of ≥ 60 J, and a corrosion rate of ≤ 0.2 g/m²·h after 120 h of 5% NaCl neutral salt spray corrosion test.

9. A manufacturing method for the chain according to any one of claims 6 to 8, wherein the manufacturing method comprises the following steps performed in sequence:
S1, smelting and casting molten steel to obtain a cast slab;
S2, heating and rolling the cast slab, wherein a reduction ratio of the cast slab is ≥ 10;
S3, forming rings and welding;
S4, performing quenching heat treatment, wherein for the quenching heat treatment, a heating temperature is 840-980 °C, preferably 850-950 °C, and a holding time is 1-4 hours, preferably 1-3 hours, followed by water cooling for quenching;
S5, performing pickling pretreatment to obtain a chain steel;
S6, hot-dip galvanizing, wherein the chain steel after the pickling pretreatment is subjected to preheating treatment followed by hot-dip galvanizing to obtain the chain comprising the chain steel and a zinc coating formed on the surface of the chain steel; a temperature difference between a preheating temperature for the preheating treatment and a temperature of zinc bath used in the hot-dip galvanizing is controlled to -30 to 30 °C.

10. The manufacturing method according to claim 9, wherein
in step S1, the smelting comprises electric furnace or converter smelting, LF refining, and VD or RH vacuum treatment; the casting is performed using a continuous casting process; preferably, the VD or RH vacuum treatment is performed for 10-20 min; during casting, a superheat degree of molten steel in tundish is controlled to 15-40 °C; and/or
in step S2, during heating and rolling, the cast slab is heated at a heating temperature of ≥ 1150 °C for a heating time of 3-6 h, and a finishing rolling temperature is ≥ 850 °C; after rolling, air cooling or slow cooling is performed; and/or
in step S6, the preheating temperature is 400-550 °C, and a preheating time is ≥ 0.5 h; the temperature of zinc bath used in the hot-dip galvanizing is 400-530 °C.

11. The manufacturing method according to claim 9, wherein the zinc coating has a thickness of 10-150 µm, preferably 40-150 µm.

12. The manufacturing method according to claim 9, wherein the chain steel in the chain obtained in step S6 has a microstructure of tempered martensite and carbides dispersed interlamellarly.

13. The manufacturing method according to claim 9, wherein the chain has the following properties: a yield strength Rp_{0.2} of ≥ 1050 MPa, a tensile strength Rₘ of ≥ 1200 MPa, an elongation A of ≥ 14%, a reduction of area Z of ≥ 50%, a Charpy impact energy Aₖᵥ at -20 °C of ≥ 60 J; and a corrosion rate of less than 0.2 g/m²·h after 120 h of 5% NaCl neutral salt spray corrosion test.
